

## UNITED STATES PATENT OFFICE

2,270,717

## PROCESS OF TRANSFERRING HEAT

Vladimir L. Shipp, New York, and John Happel,  
Brooklyn, N. Y., assignors to Socony-Vacuum  
Oil Company, Incorporated, New York, N. Y., a  
corporation of New York

No Drawing. Application May 22, 1940,  
Serial No. 336,592

3 Claims. (Cl. 252—73)

This invention has to do with the art of heating and heat transfer. It is concerned with those processes wherein a fluid medium, circulated under pressure, is heated in one portion of a cycle and utilized to deliver heat in another portion of the cycle, the whole object of the process being to deliver heat to apparatus isolated from the furnace or other means wherein the fluid medium is heated. Commercial systems of this type commonly utilize a heavy mineral oil fraction as the fluid heat transfer medium. This invention is specifically directed to such processes using oil as a heat transfer medium.

This application is a continuation in part of our copending application Serial No. 211,698, filed June 3, 1938.

The object of this invention is to provide such a process which is free from the hazards, disadvantages, and costs coincident to the degradation of the oil used as a fluid heat transfer medium.

The equipment utilized in such processes is well known and consists of a fired furnace or other type of heater in which the oil, circulating continuously, is heated to a high temperature, usually not higher than about 550° F. to about 600° F. The hot oil is circulated to the point where heat is to be applied, e. g., to the jacket of a kettle in which some reaction or process is conducted, and is then returned to the furnace.

In general, such systems have used a very heavy oil, the oil preferred heretofore being the best grade Pennsylvania or paraffinic type lubricating oil of high flash point, known to the trade as "cylinder stock." The principal requirement heretofore thought necessary for the oil was the possession of a high "flash point" believed to indicate freedom from fire risk. Such systems, using the oil heretofore recommended as best, have encountered difficulties in operation, which, while not serious at low temperatures in well designed apparatus, become crucial at higher temperatures and/or with poor design. A very important difficulty is that of a great tendency of the oil to deteriorate and become possessed of a lower flash point, and hence more susceptible to ignition and more dangerous to use. Another important difficulty is the appearance of coke, carbonaceous impurities, and sludge in such oils under use, the deposit of which greatly decreases the heat transfer capacity of the apparatus, and which necessitates continuous straining during use and promotes clogging, burning, coking, and erosion of apparatus. Another difficulty is the tendency of such oils, in use, to liberate hydrocarbon gases. All of these disadvantages may be avoided by following the teaching of this invention.

Further, present demands for extension of the field of the process to temperatures of about 60

600° F. and above are incapable of being met by the heat transferring oil now used, since oils of this type decompose quite rapidly at temperatures of this order. It must be emphasized that while the phenomenon of decomposition referred to herein is of the same nature as thermal cracking of hydrocarbon, the heat transfer oils are called upon to withstand the temperatures to which they are exposed for periods ranging into years rather than hours or minutes as in cracking.

This invention is based upon the discovery that the selection of oils upon the basis of high flash point is entirely erroneous, and that the use of oils of entirely different characteristics, as described herein, leads to entirely unexpected results and benefits in a manner contrary to the prior teaching of the art.

This invention is based upon the use of a high temperature refractory oil of a low gravity, of narrow boiling range, but not capable of producing a substantial amount of vapors at the temperature of operation, of low viscosity, and of a gas oil nature rather than of a lubricating oil nature. Such a material will have a flash point materially lower than the material heretofore used.

To contrast one such new material with that heretofore used, the following tabulation shows comparative data on a typical old-style material and a typical new material.

TABLE I

|                         | Old type | New type |
|-------------------------|----------|----------|
| Gravity A. P. I.        | 24.2     | 19.3     |
| Flash (C. Q. C.) °F.    | 590      | 310      |
| Fire °F.                | 690      | 360      |
| Visc. Saybolt Universal |          |          |
| At 100° F. seconds      |          | 79       |
| At 210° F. do           | 221      |          |
| Per cent distilled off  |          |          |
| At 400° F.              | 0        | 0        |
| At 500° F.              | 0        | 0        |

Such oils may be obtained conveniently as distillates from residual oil produced by cracking gas oil or heavier oils to gasoline. Depending upon the actual set-up of the cracking process, oils of the desired characteristics may actually emerge from the cracking equipment as a portion of the residuum there produced, as a portion of some intermediate distillate boiling between gasoline and residuum, or may be taken from such equipment by appropriate fractionation as a product ready for the present use. In all cases, however, they may be described as materials of a gas oil nature derived from hydrocarbon stocks which have been subjected to cracking, or, more shortly, as cracked mineral oil fractions having certain physical characteristics.

The refractory nature of the new type fluid heat transfer medium is well demonstrated by its superiority in use, as demonstrated by the following comparison of new and old type oils after each has been heated at 650° F. for a period of five hours under a pressure sufficient to prevent substantial vaporization.

TABLE II

|                              | Old type | New type |
|------------------------------|----------|----------|
| Gravity °A. P. I.            | 24.3     | 18.8     |
| Flash (C. O. C.)             | 590      | 320      |
| Fire                         | 665      | 360      |
| Viscosity Saybolt Universal— |          |          |
| At 100° F. seconds           | 203      | 85       |
| At 210° F. do                | 3.89     | 1.01     |
| Conradson carbon             | 2.0      | 0.0      |
| Percent distilled off—       |          |          |
| At 400° F.                   | 7.5      | 0.0      |
| At 500° F.                   |          |          |

Note that the old type oil has suffered serious degradation resulting in the formation of light, low boiling material (per cent distilled off) sufficient to materially increase the hazard attendant upon its use. It also has over three times as much carbon and sludgy material.

Of great importance is the difference in viscosity of the oils of old and new type, the new type oil having a viscosity so much lower than the old that very material savings in pumping costs are possible. Of additional interest is the fact that the oils of the new type are higher in specific heat than the oils heretofore used.

The advantages claimed for the new type of oil are capable of complete substantiation based upon actual use. In commercial operation it has been found that savings due to power and increased heat transfer efficiency amounted to 25% and that, rather than forming sludge, the new type oil was actually dissolving and freeing and removing from the system sludge and coke deposited therein by the former oil. Also, oils of the new type, after twenty months' continued use, show no appreciable changes in gravity, viscosity, color, presence of lower boiling materials, or of sludge originating from the oil.

The oils of the new type may be defined as oils which do not form material amounts of fixed gases when exposed for substantial lengths of time to elevated temperatures. For example, they may be tested for such gas formation by being heated to and held at temperatures in the range 600-700° F. in a vessel connected with a condenser, and the fixed gas noncondensable at atmospheric pressure and temperature, so formed can be collected and measured. Comparative data from such a test, carried out on an old type and a new type oil follows:

TABLE III

Rate of gas production—cubic feet/minute/100 gallons oil

| Temperature | Old type oil | New type oil |
|-------------|--------------|--------------|
| 600         | 0.7          | 0            |
| 644         | 2.1          | 0            |
| 664         | 8.9          | 0            |
| 700         | 40.2         | 0            |

From this it may be observed that these new oils may be defined as oils which are substantially resistant to thermal decomposition, as evidenced by formation of normally non-condensable gaseous products, upon prolonged ex-

posure to temperatures within the range 600-700° F. In this connection, it may be remarked that it is quite definitely established in the art of thermal decomposition of hydrocarbons that results obtained from comparatively short exposure to active cracking temperatures may be obtained also by much longer exposure to much lower temperatures. Consequently, to those skilled in the art, the above noted evolution of measurable quantities of gas in the above "old oil" at temperatures above 600° F. is a reaction of the same character as that giving sludge, coke, reduction of flash, gas evolution, and similar degradation in the "old oil" when exposed for periods of months and years to temperatures around 500-550° F.

Oils of the new type may also be defined by means of physical characteristics, the most outstanding of which is that for a given gravity, they are possessed of viscosities and boiling ranges substantially lower than those normally associated with naturally occurring mineral oil fractions of similar gravity.

A less highly indicative characteristic of such oils is their aniline point, a chemical characteristic, defined as the lowest temperature at which the oil is completely miscible with an equal volume of aniline. For comparison, a typical oil of the old type has an aniline number of 115° C., while a typical oil of the new type has an aniline number of 68° C. In general, the useful characteristics of oils of the new type with which this invention is concerned will be associated with aniline points of 80° C. or less.

Oils at present preferred for the uses above outlined will, in general fall within the range of properties outlined below:

TABLE IV

|                                                                                                                                                                                                                                                          |                  |
|----------------------------------------------------------------------------------------------------------------------------------------------------------------------------------------------------------------------------------------------------------|------------------|
| 40 Gravity °A. P. I.                                                                                                                                                                                                                                     | 0 to 30          |
| Initial boiling point, °F.                                                                                                                                                                                                                               | 575 to 850       |
| Viscosity at 100° F. (seconds)                                                                                                                                                                                                                           |                  |
| S. U. V.)                                                                                                                                                                                                                                                | 60 to 250        |
| Aniline point                                                                                                                                                                                                                                            | 80° C. or lower. |
| 45 The initial boiling point of such oils should be sufficiently high so that no generation of vapors under the conditions obtaining in the heating system will occur, and to this end, this property must be correlated somewhat with intended use. For |                  |
| 50 most present conditions, an initial boiling point of about 575° F. (A. S. T. M. method) will be sufficient, although for use at higher temperatures, this should be correspondingly higher.                                                           |                  |

We claim:

55 1. The method of applying heat at temperatures ranging from 600° F. to around 700° F. comprising continuously circulating a fluid heat transfer medium in a closed cycle, applying heat to said medium in one portion of said cycle and removing useful heat from it at another portion of the cycle, in which the fluid heat transfer medium is a cracked mineral oil fraction, substantially resistant to thermal decomposition, as evidenced by formation of normally non-condensable gaseous products, upon prolonged exposure to temperatures within the range 600-700° F. conforming to the following specification:

Gravity °A. P. I. 0 to 30  
Initial boiling point, °F. 575 to 850

70 Viscosity at 100° F., seconds  
Saybolt Universal 60 to 250  
Aniline point 80° C. or lower.

2. The method of applying heat at temperatures ranging from 600° F. to around 700° F. com-

prising continuously circulating a fluid heat transfer medium in a closed cycle, applying heat to said medium in one portion of said cycle and removing useful heat from it at another portion of the cycle, in which the fluid heat transfer medium is a cracked mineral oil fraction, substantially resistant to thermal decomposition, as evidenced by formation of normally non-condensable gaseous products, upon prolonged exposure to temperatures within the range 600-700° F., having an initial boiling point of at least 575° F., and a viscosity not greater than about 250 seconds Saybolt Universal at 100° F.

3. The method of applying heat at temperatures ranging from 600° F. to around 700° F. comprising continuously circulating a fluid heat

transfer medium in a closed cycle, applying heat to said medium in one portion of said cycle and removing useful heat from another portion of the cycle, in which the fluid heat transfer medium is a cracked mineral oil fraction of gas oil nature, having an initial boiling point of at least 575° F., and substantially resistant to thermal decomposition, as evidenced by formation of normally non-condensable gaseous products upon prolonged exposure to temperatures within the range 600-700° F., and a viscosity not greater than of the order of about 250 seconds Saybolt Universal at 100° F.

VLADIMIR L. SHIPP.  
JOHN HAPPEL.